

# UNITED STATES PATENT OFFICE.

ERICH SPRINGBORN, OF LONDON, ENGLAND, ASSIGNOR OF ONE-HALF TO  
WILLIAM MERRITT GILLAM, OF SAME PLACE.

## RELATING TO DRYING AND CONDENSING PEAT FOR FUEL OR OTHER PURPOSES.

SPECIFICATION forming part of Letters Patent No. 665,619, dated January 8, 1901.

Application filed May 15, 1900. Serial No. 16,824. (No specimens.)

*To all whom it may concern:*

Be it known that I, ERICH SPRINGBORN, analytical chemist, a subject of the Emperor of Germany, residing at 203 Burdett road, London, England, have invented certain new and useful Improvements in and Relating to Drying and Condensing Peat for Fuel or other Purposes, of which the following is a specification.

10. This invention relates to a process for drying peat for fuel or for other purposes, and has for its object to so dry such peat as to increase its density and produce a readily-combustible substance of high calorific power.
15. According to my invention I mix together about one hundred and twelve pounds of unslaked lime, about one hundred and twelve pounds of soot or powdered charred peat or similar carbonaceous substance in a finely-divided state, from one-quarter per cent. to two per cent. of sugar, and from one-quarter to one per cent. of potassium nitrate. The lime in the above mixture may be partly or wholly replaced by baryta. I add this mixture to
20. from forty to eighty times its weight of peat, the proportion of the peat to the aforesaid mixture varying as the amount of moisture in the peat. Peat usually contains from fifty-two per cent. to ninety-six per cent. of moisture. To the above specified quantity of the mixture there would therefore be added forty times its weight of peat containing sixty per cent. of moisture or eighty times its weight of peat containing seventy-five per cent. of moisture, peat containing intermediate quantities of moisture being treated with corresponding intermediate quantities of the mixture. The wet peat and the mixture are thoroughly kneaded and mixed together as intimately as
25. possible and then formed into suitable blocks and subjected to an approximately light and continuous pressure of from one-half pound to one pound per square inch for from two to four hours. The compressed blocks are then permitted to dry in drying-sheds usually for about fourteen days. It is important that but a moderate and steady pressure be exerted on the blocks for the time stated. If the pressure exceeds the amount stated, the blocks
30. cannot be subsequently dried while retaining a high specific gravity. The blocks thus ob-

tained are almost free from moisture. They have a specific gravity of about 1.3, and consequently a high calorific power. These blocks are not liable to split when drying.

55

If the pressure on the peat is too heavy, the blocks obtained have not such a high specific gravity as the blocks made according to my invention. Moreover, such heavily-pressed blocks will expand shortly after being released from the heavy pressure.

The lime or its equivalent in the mixture combines with the water in the peat, while the soot or finely-divided carbon absorbs the oil of the said peat. The sugar, in combination with the potassium nitrate, dissolves part of the lime, strengthens the action of the lime on the peat-fiber, and prevents the lime from combining with the soot, the lime and soot thus acting independently of each other and on the water and oil, respectively, and a thorough reaction being thus obtained.

In treating brown or light-brown peat which does not contain a large quantity of oils the quantity of sugar in the mixture may be greatly reduced.

65

What I claim is—

1. A process for drying and condensing peat which consists in intimately mixing the said peat with the oxid of an alkaline earth, finely-divided carbon, sugar and an alkali salt, subjecting this mixture to a moderate continuous and steady pressure, and then permitting it to dry, substantially as described.

2. A process for drying and condensing peat which consists in mixing together an oxid of an alkaline earth, finely-divided carbon, sugar and an alkali salt, then adding this mixture to the peat, then forming the total mixture into blocks and subjecting it to a moderate continuous and steady pressure, and then permitting the mixture to dry, substantially as described.

3. A process for drying and condensing peat which consists in mixing together, lime, soot, sugar and nitrate of potash, then adding this mixture to the peat, then subjecting the total mixture to a moderate continuous and steady pressure, and then permitting the said mixture to dry, substantially as described.

4. A process for drying and condensing peat which consists in combining the moisture of

70

75

80

85

90

95

100

the peat with a mixture of an oxid of an alkaline earth, an alkali salt and sugar, absorbing the oil of the peat with finely-divided carbon, then subjecting the total mixture to a moderate, steady, and continuous pressure to drive away excess of moisture, and then permitting the mixture to dry, substantially as described.

5. A process for drying and condensing peat which consists in adding a mixture of one hundred and twelve pounds of an oxid of an alkaline earth, one hundred and twelve pounds of finely-divided carbon, from one-quarter per cent. to two per cent. of sugar, and from one-quarter per cent. to one per cent. of nitrate of potash, to from forty to eighty times its weight of the moist peat, then subjecting the total mixture to a steady and continuous pressure

of from half a pound to one pound per square inch, and then permitting the mixture to dry, substantially as described.

6. Dried condensed substance consisting of peat with an oxid of an alkaline earth, finely-divided carbon, sugar, and an alkali salt substantially as described.

7. Dried condensed substance consisting of peat with unslaked lime, soot, sugar, and nitrate of potash, substantially as described.

In testimony whereof I have hereunto set my hand, in presence of two subscribing witnesses, this 4th day of May, 1900.

ERICH SPRINGBORN.

Witnesses:

F. J. SHERRINGTON,  
WALTER J. SKERTEN.